

# UNITED STATES PATENT OFFICE.

HERBERT GRAY TORREY, OF STIRLING, NEW JERSEY.

## ALLOY FOR BEARINGS, &c.

SPECIFICATION forming part of Letters Patent No. 635,615, dated October 24, 1899.

Application filed June 29, 1899. Serial No. 722,815. (No specimens.)

*To all whom it may concern:*

Be it known that I, HERBERT GRAY TORREY, of Stirling, in the county of Morris, and in the State of New Jersey, have invented certain new and useful Improvements in Alloys for Bearings, &c.; and I do hereby declare that the following is a full, clear, and exact description thereof.

The object of my invention is to provide a satisfactory antifriction alloy for journal-bearings, steps, &c., of such strength as to be capable of withstanding great strains and especially adapted for shafts that run at high speed; and to this end said invention consists in the alloy having the composition substantially as hereinafter specified.

My alloy is made of the following metals in proportion within the limits stated, to wit: lead, five hundred to eight hundred and fifty parts; antimony, one hundred to one hundred and sixty parts; tin, twenty-five to fifty parts, and cadmium one to sixteen parts. The proportions I prefer, expressed approximately, are, lead, seven hundred and ninety-five parts; antimony, one hundred and fifty-five parts; tin, forty-seven and one-half parts, and cadmium two and one-half parts. I of course do not restrict myself to the proportions mentioned, as variations may be and are made according to the use for which the alloy is designed.

In making my alloy the lead and antimony are melted together and thoroughly stirred

while melting, the oxids being disposed of by being skimmed off or by the use of some reducing agent, such as rosin. The tin should then be added, and finally the cadmium, the latter being put in just before the alloy is cast.

While I have designed my alloy for use as a bearing, I of course do not restrict myself to this use of it.

Having thus described my invention, what I claim is—

1. An alloy in which are combined lead, antimony and cadmium.

2. An alloy in which are combined lead, antimony, tin and cadmium.

3. An alloy in which are combined lead, between five hundred and eight hundred parts; antimony, between one hundred and one hundred and sixty parts; tin, between twenty-five and fifty parts; and cadmium, between one and sixteen parts.

4. An alloy in which are combined, lead, seven hundred and ninety parts; antimony, one hundred and fifty-five parts; tin, forty-seven and one-half parts; and cadmium, two and one-half parts.

In testimony that I claim the foregoing I have hereunto set my hand this 14th day of June, A. D. 1899.

HERBERT GRAY TORREY.

Witnesses:

CHARLES BENNER,  
JOHN E. ROESER.